

## UNITED STATES PATENT OFFICE

1,934,586

MATERIAL FOR PARTS SUBJECTED TO  
FRICTION

Oskar Brandenberger, Zurich, Switzerland

No Drawing. Application March 20, 1930, Serial  
No. 437,611, and in Germany July 17, 1929

2 Claims. (Cl. 308—242)

This invention relates to parts subjected to friction, such as bearings and the like, and its object is to provide an improved material for parts subjected to friction, or bearings, said parts or bearings being formed according to the invention of copper alloy containing sulphur, notably bronze or red metal alloy containing up to 4% of sulphur. Such bronze or alloy is a Cu-Sn-Zn-alloy, designated as "red metal" and given under "Rotguss" in Din. The word Din is the accepted 5 abbreviation for the German words corresponding to the English "German Industry Standards".

Under the term Rotguss are to be understood alloys of copper with tin and zinc, with or without the addition of lead and other impurities. The 10 best known Rotgusses are: the German "Eisenbahn-Rotguss Rg 9", containing 85% copper, 9% tin and 6% zinc; Rotguss Rg 5 containing 85% copper, 5% tin, 7% zinc and 3% lead; and Rotguss Rg 10 (machine bronze) containing 86% copper, 20 10% tin and 4% zinc.

As a result of the addition of sulphur the anti-friction properties of the alloy are much improved and the hardness and lasting properties thereof are increased, whilst any tendency towards porosity is diminished.

It is not always advisable that the sulphur content of the material should exceed 4%, as with some alloys when the sulphur content exceeds 4% a copper matte product rich in sulphur is liable 25 to be formed, said product, if formed, separating out from and floating on the molten alloy owing to its lower specific gravity.

The sulphur may be added to the alloy either in an uncombined state or as a sulphur compound. As a result of this addition, chiefly cop-

per sulphide ( $Cu_2S$ ) is formed in bronze and red metal alloys, said sulphide being slightly soluble in a liquid state in the liquid alloy, but practically insoluble in the solidified alloy and occurring as a separate ingredient in the form of evenly dispersed small roundish embedded particles. As 60 well as giving rise to the formation of copper sulphide, the addition of sulphur influences the normal structure of certain bronze and red metal alloys. For example, in tin bronzes the quantity of eutectoid is considerably diminished with increasing sulphur content.

The improvement in the anti-friction properties of bronze and red metal alloys by the addition of sulphur is very marked. Moreover, bearing surfaces of sulphur bronze have three to four 70 times the working life of those made from alloy without sulphur but otherwise of the same composition. Not only is the wearing away of sulphur bronze alloys considerably less than that of similar alloys without sulphur, but bearings made 75 from such sulphur bronze alloys can be submitted to considerably greater surface pressure. The coefficient of friction of sulphur bronze alloy is considerably less than that of similar alloys without sulphur.

What I claim is:—

1. A bearing metal mostly consisting of copper, tin, zinc, lead and up to 4% sulphur with a major proportion of copper.
2. A bearing made of an alloy of the bronze 85 and red brass type, mostly consisting of copper, tin, zinc, lead and up to 4% sulphur with a major proportion of copper.

OSKAR BRANDENBERGER.

90

40

95

45

100

50

105

55

110